

Sept. 6, 1938.

L. J. WILLIEN ET AL

2,129,341

PROCESS OF MANUFACTURING CARBURETED WATER GAS

Filed Aug. 3, 1928



FIG. 1



FIG. 2



FIG. 3

Inventors  
Leon J. Willien,  
and Louis Stein,  
By Forbes Silby  
ATTORNEY

## UNITED STATES PATENT OFFICE

2,129,341

## PROCESS OF MANUFACTURING CARBURETED WATER GAS

Leon J. Willien, Chicago, Ill., and Louis Stein, Minneapolis, Minn., assignors to The United Gas Improvement Company, Philadelphia, Pa., a corporation of Pennsylvania

Application August 3, 1928, Serial No. 297,243

3 Claims. (Cl. 48—208)

This invention relates to the production of combustible gas and more particularly to a process and apparatus for making carbureted water gas. This application is a continuation in part 5 of our prior application Serial No. 187,876, filed April 30, 1927.

One object of this invention is to provide a process for manufacturing carbureted blue water gas such as is commonly used for illuminating, 10 heating and various other purposes, having a substantially lower specific gravity than is commonly obtainable by the practice of present processes.

Another object of this invention is to provide a process for making carbureted water gas which may be practiced in existing gas-making sets comprising a generator, carburetor, superheater and wash box connected in series, or in existing sets that can readily and easily be modified for 20 the purpose of practicing our invention. By the practice of this process there is periodically obtained a higher B. t. u. gas and/or more gas so that irregular, temporary, peak or unusual demands for gas from a given gas installation may be met without the use of a spare installation or 25 additional equipment, or without having the gas set of greater capacity than that required for normal operation. Accordingly, by the practice of our process, there is effected an economy in the equipment necessary for generating gas to 30 meet both the usual and unusual demands therefor.

Our invention involves an improvement in the process of making carbureted water gas in a three-shell set including a generator, carburetor and superheater, which comprises a blast to heat the fuel bed to incandescence and store heat in the carburetor and superheater, one combustible gas-making run wherein steam is passed through the fuel bed of the generator and the resultant 40 gas passed into and through the carburetor where it is enriched with the customary oil, namely petroleum oil, the enriched gas being passed into and through the superheater and wash box 45 and the usual purifying and gas treating devices into a holder, and a second combustible gas generating run commonly known as the back-run, consisting in introducing steam at any convenient point into the set, preferably into the superheater, 50 and then passing the steam through the set into the generator and through the fuel bed therein, the resultant gas being passed into the wash box and thence into and through the purifying 55 and gas treating devices and usually admixed with the combustible gas made in a previous cycle. According to such processes, carbureted water gas of a B. t. u. value equal to the mean B. t. u. value of the gas obtained from both combustible 60 gas generating runs of the cycle is produced and

a substantially constant volume of gas is generated by the gas-making set.

According to the present invention, oil of the above type is added to the steam passing through the superheater and carburetor prior to passage 5 thereof through the fuel bed in the generator, the resultant mixture being passed through the fuel bed and the resultant gas passed directly from the generator to the wash box. The oil may be introduced into the superheater simultaneously 10 with the introduction of steam thereinto. By the practice of our process carbureted water gas of a greater B. t. u. value, low gravity gas and/or a greater yield of gas is obtainable.

In the operation of water gas sets there are 15 frequent temporary demands for increased gas and heretofore, to accommodate such demands, it has been necessary to provide a spare installation for the generation of the increased gas to meet such temporary demands or peak loads. 20 According to our invention, carbureted water gas sets are operated as is customary to meet the normal demands but when it is necessary to generate more gas to accommodate increased or peak demands in enriching constituent such as 25 oil, as hereinbefore pointed out, is added to the gas-making steam of the back run, for example introduced into the superheater and the mixture of steam and oil is passed into and through the fuel bed in the generator down through the fuel 30 bed so that more gas and/or gas of higher B. t. u. value is producible. It will be noted that according to our invention, it is possible to meet the incidental and irregular or temporary demands 35 for increased gas without having a spare installation, or without having a gas set with a greater capacity than that required for normal operation.

In the accompanying drawing there has been 40 disclosed a structure designed to carry out the various objects of the invention, but it is to be understood that the invention is not confined to the exact features shown, as various changes 45 may be made within the scope of the claims which follow.

In the accompanying drawing forming part of 45 this specification:

Figure 1 is a vertical sectional view of a form of apparatus for manufacturing carbureted blue water gas, showing the invention applied thereto; 50

Figure 2 is a sectional plan view on the line 2—2 of Figure 1; and

Figure 3 is an enlarged detailed sectional view on the line 3—3 of Figure 2, showing a form of oil spray nozzle.

The gas manufacturing apparatus illustrated in Figure 1 comprises the usual water gas generator 5, carburetor 6, and the superheater 7. The water gas generator and carburetor are connected together by means of a pipe 8 and the 60

carburetor and superheater are similarly connected together at their lower portions by means of a conduit 9. The carburetor and superheater have provided therein the usual checker brick 11, 5 as is customary in structures of this kind. A grate 12 is provided in the generator 5 beneath which is the usual ash pit 13, having an air supply pipe 14 connected therewith for blasting the fuel bed. A valve 15 controls the flow of air to the 10 generator. A steam pipe 16 is also connected with the ash pit 13 and has a control valve 17 for regulating the flow of steam delivered to the apparatus during the process of making the gas.

A gas take-off connection 18 is provided at the 15 upper end of the superheater 7 and has one end connected with a valve mechanism, such as the three-way valve 19, shown in Figure 1, for controlling the flow of gas from the superheater to the usual wash box 21. This wash box has a 20 connection 22 leading to a suitable gas storage means, not shown. A connection 23 connects the three-way valve 19 with the ash pit 13 of the generator. A valved steam intake pipe 24 is also provided in the gas take-off 18, whereby the gaseous flow through the apparatus may be reversed, 25 as will subsequently be described. The superheater is further provided with the usual stack valve 25, which is opened during the air blasting operation of the fuel bed and is closed during 30 the gas-making portion of each cycle of operation. The usual oil spray nozzle 26 is shown mounted in the upper portion of the carburetor 6, and a fuel door 27 is provided in the top of the generator for fueling the generator when necessary.

35 In a gas manufacturing set or apparatus, such as above described, steam is introduced into the generator from the pipe 16, after the fuel bed has been blasted in the usual manner and the checker-brick 11 in the carburetor and superheater have 40 been heated to the desired temperatures. The steam, in passing through the incandescent fuel bed, is decomposed and forms water gas which passes through the connection 8 into the upper portion of the carburetor, thence downwardly 45 through the checker-brick therein, and through the connection 9 into the bottom of the superheater. From the bottom of the superheater the water gas passes upwardly through the checker-brick therein and is discharged therefrom through 50 the gas take-off 18, into the wash box 21, from which it passes through the pipe 22 to a suitable storage means, such as a relief holder, not shown. In order to produce a carbureted blue water gas that is adapted for use for commercial purposes, 55 it is necessary that the gases in the apparatus, before reaching the wash box 21, be enriched by a suitable enriching fluid, such as oil, for the purpose of increasing the calorific value of the resultant gas. In the usual process of manufacturing 60 carbureted blue water gas, as above described, oil is introduced into the apparatus, usually at the top of the carburetor, by means of the oil spray nozzle 26 and after the steam has passed through the generator fuel bed and water gas has been 65 formed, the oil is added to the water gas while passing through the carburetor.

The type of apparatus illustrated in Figure 1 is of the up-and-down or back-run type, wherein the flow of steam or gases through the apparatus 70 may be reversed, that is, for the up-run the steam is introduced into the apparatus in the lower portion of the generator, and is discharged in the form of gas through the take-off 18 at the upper portion of the superheater. After the up-run flow 75 of steam has continued for a predetermined peri-

od of time, the supply of steam to the generator is shut off, and the three-way valve 19 is moved to the dotted line position shown in Figure 1, to close the gas take-off 18. Steam is then preferably introduced into the upper portion of the superheater from the pipe 24, and flows downwardly through the superheater, thence upwardly through the carburetor and over into the generator and down through the fuel bed therein, and thereby generating water gas which passes into 10 the ash pit, from which it flows through the connection 23, back to the three-way valve 19, and into the wash box 21. It is understood that the steam may be introduced at any point in the set prior to the fuel bed. The above described operation is commonly known as the back-run method of operation. In the above described process of manufacturing carbureted water gas, oil is not introduced into the gases during the back-run or 15 analogous run of the gas-making operation, but during the up-run and subsequent to the passage of the steam through the fuel bed. We have found, however, from actual experimenting, that by introducing an enriching fluid, preferably oil, into the gases, prior to their passage through the 20 generator fuel bed, the hydrogen content of the resultant gas is increased, thereby lowering the specific gravity of the gas and increasing the volume of gas generated so that more gas is produced. The improved process featured in this 25 invention consists in thus introducing into the gases, prior to their passage through the generator fuel bed, a suitable enriching fluid.

In order to carry out our invention we mount 30 one or more spray nozzles 28, such as in the upper portion of the superheater wall, as shown in Figure 1. When a plurality of oil spray nozzles 28 are employed, they are preferably connected, as shown in Figure 2, to obtain their supply of oil from a pipe 29, having a connection 35 with a suitable source of supply, not shown. A control valve 31 may be interposed in the pipe 29 for controlling the flow of oil to the nozzles. The oil spray nozzles shown in the drawing are 40 of the injector type, having a connection with a steam pipe 32, connected with a supply pipe 33, having a connection with a steam source, not shown. A valve 34 is provided in the supply pipe 33 for controlling the supply of steam to the nozzles 28. Figures 2 and 3 illustrate a conventional form of oil spray nozzle of the injector type, in which the small pipe 35 is connected with the oil supply pipe 29 by means of a pipe 36. The relatively large pipe 37 communicates with the steam pipe 33. Thus, when the valve 45 50 55 60 65 70 75 80 85 90 95 99 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940

form a low gravity, carbureted blue water gas which is passed through the usual gas treating and purifying device into the holder where it is admixed with the gas produced during the preceding gas-making run. Inasmuch as there is produced in the back run, hydrogen and carbureted blue water gas, it follows that the hydrocarbon oil is not completely decomposed but is partially decomposed or cracked into hydrogen and volatile hydrocarbons or fixed oil gas by means of which the blue water gas, simultaneously generated, is carbureted. By the practice of our process there is obtainable a higher B. t. u. gas and/or more gas and the gas produced during the back run is of lower specific gravity than the gas produced when steam alone is employed during this run.

In the drawing we have also shown an oil spray nozzle 38 mounted in the upper portion of the generator so that, if desired, oil may also be introduced at this point. In some instances, it may be found desirable to introduce a portion of the oil in the superheater and a portion in the generator, or it may be found desirable to introduce all of the oil in the upper portion of the generator. In each case, however, the oil must be introduced into the steam, prior to their passage through the generator fuel bed.

It is well known that the demand for gas from a given gas installation is not constant over a period of time such as a day or more. The loads or demands for gas from given gas installations fluctuate, there being a substantially constant demand throughout the major portion of the period and demands for more or increased gas at intervals during such period of time. Heretofore, to meet such demands for increased gas or peak loads it has been the practice to operate a certain number of sets of the installations substantially continuously and at full or normal capacity to meet the normal or substantially constant demands and to maintain other spare or additional sets which were operated only at certain intervals to generate additional gas to accommodate the peak loads. By the practice of our invention, as herein disclosed, the necessity for such additional sets is eliminated and all the combustible gas equipment is operated efficiently, economically and substantially continuously to meet both normal loads and peak or increased demands for gas.

From the foregoing it will be seen that when our invention is employed, the gas made during the back-run is of lower specific gravity than either the carbureted water gas made during the up-run, or blue water gas made during a back-run when our invention is not employed. Therefore, the term "low specific gravity" refers more particularly to gas made during the back-run when our invention is employed than to the mixed gas in the holder which, as will be readily seen, may or may not be of low gravity depending upon the relative amounts of the various gases present. In any event, however, and provided all other conditions remain the same, the holder gas is of lower specific gravity than it would be if our invention were not employed.

We use the term "oil" in the specification in the way that it has heretofore been universally used in the gas industry, namely to mean "petroleum oil", that is crude oil or a fraction obtained in the refining thereof, such as petroleum naphtha, gas oil, residuum oil, and the crudes

and fractions known commercially as heavy oil. The term "petroleum oil" as used in the claims specifically excludes other hydrocarbon oil such as tar.

We claim:

1. The process of making carbureted water gas of low specific gravity, which, when practiced in a set including a single generator, a single carburetor, a single superheater, in individual detached shells, and a wash box, connected in series, comprises internally preheating the carburetor and superheater solely by air blast gas from the generator, making carbureted water gas by forward steaming and carbureting, introducing petroleum oil into the back run steam, and generating gas comprising carbureted water gas and hydrogen and of lower specific gravity than the forward run carbureted water gas and of lower specific gravity than would be the case in the absence of the introduction of the petroleum oil by passing the mixture of steam and oil down through the fuel bed partially decomposing the petroleum oil to hydrogen and to oil gas which latter carburets the water gas simultaneously generated in the fuel bed.

2. In a process for making carbureted water gas, which, when practiced in a carbureted water gas set comprising a single generator a single carburetor and a single superheater in individual detached shells and connected in series, includes a blast for bringing the fuel bed up to temperature and for heating the set, an up-run with steam during which petroleum oil is introduced into said set for carbureting the up-run water gas, and a back-run during which steam is passed in a reverse direction through said set, the step of introducing petroleum oil into said set during said back-run for passage through the fuel bed along with the steam whereby said petroleum oil is decomposed to hydrogen and hydrocarbon gas for carbureting the back-run water gas, the extent of decomposition of said last mentioned petroleum oil being such as to make the back-run gas of lower specific gravity than said up-run carbureted water gas and of lower specific gravity than would be the case in the absence of the introduction of petroleum oil into said set during said back-run.

3. A process for making carbureted water gas in a carbureted water gas set, comprising a single generator a single carburetor and a single superheater in individual detached shells and connected in series, which includes in a cycle the following steps, a blast for bringing the fuel bed up to temperature and for heating the set, an up-run with steam during which petroleum oil is introduced into said set for carbureting the up-run water gas, a back-run with steam during which petroleum oil is introduced into said set for carbureting the back-run water gas, said last mentioned petroleum oil passing through the fuel bed wherein it is decomposed to a considerably greater extent than said first mentioned petroleum oil so as to make the back-run gas of lower specific gravity than the up-run carbureted water gas and of lower specific gravity than would be the case in the absence of the introduction of petroleum oil into said set during said back-run, and then combining said up-run carbureted water gas and said back-run carbureted water gas.

LEON J. WILLIEN.  
LOUIS STEIN.